

# UNITED STATES PATENT OFFICE.

ANTON MANHART, OF VIENNA, AUSTRIA.

## ALLOYS OF ALUMINIUM AND PROCESS OF PRODUCING THE SAME.

•1,422,591.

Specification of Letters Patent. Patented July 11, 1922.

No Drawing.

Application filed August 12, 1920. Serial No. 403,156.

To all whom it may concern:

Be it known that I, ANTON MANHART, citizen of the Republic of Austria, and resident of Vienna, Clementinengasse 11, Austria, have invented certain new and useful Improvements in Alloys of Aluminium and Processes of Producing the Same, of which the following is a specification.

Alloys of aluminium which contain copper, 10 tin, antimony and magnesium besides aluminium are already known and a typical representative of this group has been described in the specification of Austrian Letters Patent No. 5842.

15 This Austrian patent describes an aluminium alloy made of the following:

100 parts of aluminum.  
12.05 parts of tin.  
0.20 parts of antimony.  
0.09 parts of phosphorus.  
7.50 parts of copper.  
0.06 parts of magnesium.  
0.06 parts of sodium carbonate or potash.  
0.04 parts of sulphur.

25 The above preparations are by weight and this alloy is made as follows:—

The tin, antimony, phosphorus, copper and magnesium are melted together and the aluminium is then added and brought to a 30 melting point. When the entire mass has melted and has been mixed, the potash and the sulphur are added and the mass is further heated.

This above described alloy, can be worked 35 easily and is exceedingly resistant against acids and oxidizing agents but it softens and therefore cannot be employed for cooking vessels. It is true, the hardness of the alloy can be increased by adding a greater quantity of copper and antimony but, as is stated in the aforementioned patent, the brittleness of the alloy is thus increased and this is undesirable.

According to my invention a part of the 45 copper is substituted by manganese-copper to such extent that the amount of copper present in the alloy is double the amount of manganese-copper.

Manganese copper in this specification 50 means an alloy of copper and manganese which has been known for more than fifty years and which can be manufactured by alloying the two metals by any approved and

well known method or by melting copper with ferro-manganese.

The percentage of manganese in such an alloy could be varied within wide limits as is well known to the art, and my invention is not limited to any particular percentage of manganese as alloys containing widely 60 variable quantities of manganese are suitable for my purpose.

Of course, the potash and sulphur are not ingredients of the alloy as finally produced.

The alloys made according to the present 65 invention are distinguished from those described in Austrian Patent No. 5842 in that aluminium is present in great excess in the alloy described in the said Austrian patent, while according to the present invention, the 70 aluminium is only about 50% of the entire composition.

As clearing agent, preferably potash ( $K_2CO_3$ ) is used.

Alloys of the best qualities have been obtained by using the following proportions:

|                  | Parts. |
|------------------|--------|
| Copper           | 2.500  |
| Manganese-copper | 1.250  |
| Tin              | 6.000  |
| Antimony         | 0.1652 |
| Magnesium        | 0.0375 |
| Potash           | 0.0375 |
| Sulphur          | 0.0125 |
| Aluminum         | 10.000 |

Naturally I do not limit myself exactly to these proportions as they may be varied to some extent according to the special purpose.

Alloys made according to my invention 90 are not brittle. They are so hard that cooking vessels can be made out of them by casting as well as out of plates of the alloy.

I claim:

1. A hard, non-brittle, castable aluminum 95 alloy having manganese, copper and tin as ingredients thereof, the amount of the aluminium present in the said alloy being in excess of the amount present of any other ingredient of the said alloy.

2. A hard, non-brittle, castable aluminum 100 alloy having copper, manganese, tin, antimony, and magnesium as ingredients thereof, substantially as and for the purposes described.

3. A hard, non-brittle, castable aluminum

55

65

75

80

85

100

105

alloy made of copper, manganese, tin, antimony, magnesium and aluminum, the amount of aluminum being substantially the same as the total amount of the other ingredients, 5 substantially as and for the purposes described.

4. A hard, non-brittle, castable aluminum alloy composed substantially of 10 parts of

aluminum, .0375 parts of magnesium, .1652 parts of antimony, 6 parts of tin, 2.5 parts of copper and less than 1.250 parts of manganese.

Signed at Vienna, Austria, this 19th day of July, A. D. 1920.

**ANTON MANHART.**